

June 12, 1928.

1,673,533

E. A. RUDIGIER

ART OF MAKING ASPHALT

Filed Aug. 19, 1922



EDWARD A. RUDIGIER  
By his Attorney  
O. G. Messenger

## UNITED STATES PATENT OFFICE.

EDWARD A. RUDIGIER, OF BALTIMORE, MARYLAND, ASSIGNOR TO STANDARD OIL DEVELOPMENT COMPANY, A CORPORATION OF DELAWARE.

## ART OF MAKING ASPHALT.

Application filed August 19, 1922. Serial No. 582,903.

My invention relates to the art of making asphalt and will be fully understood from the following description taken in connection with the accompanying drawing, which 5 represents a vertical section through one form of apparatus contemplated in the invention.

In the customary practice, asphalt is made by prolonged blowing of air through a body 10 of asphaltic oil residuum heated in a still. This not only ties up expensive still equipment designed primarily for distillation use, but the maintenance costs are high and the output efficiency is low.

15 In accordance with the present invention, the oxidation is carried on in such manner as to utilize the heat of reaction, and an illustrative form of apparatus which may be employed is shown for example in the 20 drawing, the reference character 1 designating a tank lagged with heat-insulating material 2, and having an air-pipe system comprising, for example, a manifold 3 and branches 3' therefrom provided with 25 perforations. At the top of the tank is an off-take 4 for volatile matters and residual air, such off-take, in the form shown, discharging into the base of a tower 5, which may be empty but preferably contains a suitable 30 checkerwork or loose filling, at the top of which is a spray-head 6 and thereabove in the stack further sprinklers 7 all fed from the water-pump 8 through the pipe 9.

Any usual or desired pump-line connection, as indicated at 15, may be provided for feed and discharge of the tank, the precise detail not being material.

In operation, heavy asphaltic residuum, 40 as for example Mexican petroleum which has been reduced in a continuous still battery to the extent desired, for example about 380° F. Flash, is passed while hot, through a cooling coil if necessary, into the tank so as to obtain a charge temperature of about 45 420°-440° F. Air is then admitted at a pressure, for instance, of 11-12 lbs. gauge and bubbles out from the perforated pipes and up through the body of oil. As an illustration, in one instance where a tank 50 25 feet in diameter by 30 feet high was used,

the air was delivered at a rate of 900 to 1000 cubic feet per minute, and the blowing was continued for 38 hours. The temperature of the oil, which was at 420° F. at the start, gradually rose somewhat during the 55 run and then receded to about 456° F. at the finish, the heat throughout the run being supplied by the oxidation reaction itself, since as seen, the tank is insulated against transmission of heat from without and loss 60 of heat from within.

With a view to the best quality of product, it is desirable that care be exercised to maintain a proper rate of air feed throughout the run so as to avoid temperature extremes 65 that would preclude obtaining the desired melting point and penetration for the finished product.

If it be desired, the feed air can be heated in a suitable heater or exchanger, as indicated at 12. Under ordinary conditions, however, this is unnecessary where starting with sufficiently hot oil and where heating of the air is not required, the air can be wholly or partially by-passed from supply- 70 pipe 14 through pipe 13 around the heater 12.

The vapors and fumes from the tank are advantageously passed through the tower 5 and are washed by a water spray, the wash 80 water with entrained condensate flowing down through a hydraulic seal 10 and thence by a pipe 11 to a separator so as to enable recovery of hydrocarbons.

While in describing my invention, I have 85 referred to certain specific details, it will be understood that these are illustrative and in no sense limitative; nor is the invention to be understood as dependent upon the accuracy of any theory or reasons suggested 90 in explanation of the advantageous results. On the contrary, the invention is to be regarded as limited only as defined in the following claims, in which it is my intention to claim all inherent novelty as broadly as 95 the prior art permits.

What I claim is:

1. The improvement in the art of making asphalt, which comprises distilling petroleum down to residuum in reducing stills, 100

transferring the residuum with a temperature of around 420° F., from the reducing stills to a heat insulated container, and blowing air through the collected residuum without applying external heat, to obtain the desired asphaltic characteristics.

2. The improvement in the art of making asphalt, which comprises distilling petro-

leum down to residuum in reducing stills, transferring the residuum while hot to an unheated insulated container, and maintaining the temperature of said residuum at a desired point by blowing air through the residuum.

EDWARD A. RUDIGIER.